# EUROPEAN PATENT SPECIFICATION

(11) **EP 0 808 387 B1**
(45) Date of publication and mention of the grant of the patent: **16.04.2003**
(21) Application number: 96905286.9
(22) Date of filing: 26.01.1996
(51) Int. Cl.: D21F 11/14

(54) **METHOD FOR MAKING UNCREPED THROUGHDRIED TISSUE PRODUCTS WITHOUT AN OPEN DRAW**
VERFAHREN ZUR HERSTELLUNG VON UNGEKREPPTEN, DURCHBLASGETROCKNETEN TISSUEPRODUKTEN UNTER VERMEIDUNG EINES OFFENEN ZUGES
PROCEDE DE FABRICATION DE TISSU NON CREPE SECHE A L'AIR TRAVERSANT SANS UN TIRAGE OUVERT

(30) Priority: 06.02.1995 US 384307; 06.02.1995 US 384306
(43) Date of publication of application: 26.11.1997
(73) Proprietor: KIMBERLY-CLARK WORLDWIDE, INC., Neenah, Wisconsin 54956 (US)
(72) Inventor: RUGOWSKI, James, Sigward, Appleton, WI 54915 (US); REKOSKE, Michael, John, Appleton, WI 54914 (US); LIN, Philip, Sim, Tulsa, OK 74105 (US); GROPP, Ronald, Frederick, St. Catharines, Ontario L2N 2T8 (CA); ARNOLD, Paul, André, Benoît, Luc, M., F-54460 Liverdun (FR)
(74) Representative: DIEHL GLAESER HILTL & PARTNER
(86) International application number: US9601244
(87) International publication number: WO96024718

(56) References cited:
- EP-A- 0 617 164
- WO-A-81/02704
- GB-A- 1 389 992
- US-A- 4 356 059
- US-A- 4 440 597

## Description

### Background of the Invention

In the manufacture of tissue products such as facial tissues, bath tissues and paper towels, the tissue basesheets are generally produced by depositing an aqueous suspension of papermaking fibers onto a forming fabric, dewatering the suspension to form a web, drying the web, and winding the dried web into a roll for subsequent conversion into a particular product form. During manufacturing, most tissue webs are adhered to a steam-heated Yankee dryer and thereafter dislodged from the surface of the Yankee by contact with a doctor blade (creping) prior to converting to improve the softness and stretch of the sheet. More recently, soft uncreped throughdried tissue sheets have been disclosed in which the softness and stretch are built into the sheet by other processing methods.

However, in all such processes, the final sheet traverses an "open draw" before being wound into rolls, meaning that the dried sheet is momentarily unsupported before being wound. In the case of creped sheets, the sheet is dislodged from the creping cylinder and passed unsupported from the creping cylinder to the reel. For uncreped throughdried sheets, the sheet leaves the throughdrying fabric, or a subsequent transfer fabric, and also passes unsupported to the reel. As those in the tissue manufacturing business know, these unsupported runs or open draws are a source of sheet breaks and production delay time. To compensate, the tissue sheets are designed to have high machine direction strengths in order to remain intact during manufacturing. However, such high strengths are often counterproductive in terms of softness and are not desirable to the end user of the product.

Therefore, if open draws in tissue manufacturing could be eliminated, tissues could be made more efficiently from a waste-and-delay standpoint and the machine direction strength of the final product could be reduced to levels dictated solely by product requirements rather than manufacturing requirements.

EP-A-0 617 164 relates to an uncreped throughdried cellulosic web having high smoothness and stretch, which is produced by transferring a newly formed web from the forming fabric to a slower moving, high fiber support transport fabric, transferring the web to a throughdrying fabric and throughdrying the web to a final dryness. Before being wound onto the reel, the web transverses an open draw.

WO-A-81/02704 relates to a method for making a creped throughdried tissue, and a paper machine in which the web can be transferred all the way up to the reeling means in a no-draw conduction.

### Summary of the Invention

It has now been discovered that in the manufacture of uncreped throughdried tissue sheets, the open draw between the throughdryer and the reel can be eliminated using an appropriate combination of dry end transfer fabrics and/or other transfer devices. In so doing, tissue sheets having much lower machine direction strengths can be made, thereby providing a means for making tissue sheets that are softer and more "square" in terms of the machine direction and cross-machine direction tensile strengths.

Subject matter of the present invention is a method for making an uncreped throughdried tissue as claimed in claims 1 and 4, and a papermaking machine for continuously making an uncreped throughdried paper web as claimed in claims 9 and 10. The dependent claims relate to preferred embodiments thereof.

Hence in one aspect, the invention relates to a method for making an uncreped throughdried tissue comprising depositing an aqueous suspension of papermaking fibers onto a forming fabric to form a wet web, transferring the wet web to a throughdrying fabric, throughdrying the web to form a tissue sheet, and transferring the tissue sheet to a reel such that the sheet does not traverse an open draw while being wound onto the reel in the winding nip formed between the reel and a reel drum. Avoidance of the open draw is achieved either by an intermediate transfer to dry end transfer fabrics. This method is particularly advantageous at high machine speeds (about 2000 or about 3000 feet per minute or greater) where a relatively high MD tensile strength is otherwise necessary for the sheet to pass to the reel without periodically breaking.

Hence in one embodiment, the invention resides in the foregoing method wherein the tissue sheet is: (a) transferred from the throughdrying fabric to a first dry end transfer fabric using a vacuum roll; (b) carried between the first dry end transfer fabric and the top side of a second dry end transfer fabric having a relatively high degree of air permeability about 60 m³ per minute per m² (about 200 cubic feet per minute per square foot)or greater), the underside of which partially wraps around the reel drum; (c) transferred to the top side the second dry end transfer fabric and maintained thereon by air pressure created by an air foil positioned on the underside of the second dry end transfer fabric; and (d) wound onto the reel. More specifically, the air permeability of the second dry end transfer fabric can be from about 60 to about 150 m³ per minute per m² (about 200 to about 500 cubic feet per minute per square foot), still more specifically from about 90 to about 120 m³ per minute per m² (about 300 to about 400 cubic feet per minute per square foot). Air permeability, which is the air flow through a fabric while maintaining a differential air pressure of 1.27 cm (0.5 inch) across the fabric, is described in ASTM test method D737.

In another embodiment, the invention resides in the foregoing method wherein the tissue sheet is: (a) transferred from the throughdrying fabric to a first dry end transfer fabric using a vacuum roll; (b) carried between the first dry end transfer fabric and the top side of a second dry end transfer fabric having an air permeability of about 30 m³ per minute per m² (about 100 cubic feet per minute per square foot)or less, the underside of which partially wraps around the reel drum; (c) transferred to the top side the second dry end transfer fabric; and (d) wound onto the reel. More specifically, the air permeability of the second dry end transfer fabric can be from 0 to about 30 m³ per minute per m² (0 to about 100 cubic feet per minute per square foot), more specifically from about 7.5 to about 30 m³ per minute per m² (about 25 to about 100 cubic feet per minute) per square foot, still more specifically from about 15 to about 30 m³ per minute per m² (about 50 to about 100 cubic feet) per minute per square foot.

In another aspect, the invention relates to a papermaking machine for continuously making uncreped throughdried paper webs comprising:
(a) a headbox for depositing an aqueous suspension of papermaking fibers onto a forming wire; (b) a continuous forming fabric for receiving the aqueous suspension of papermaking fibers to form a wet web; (c) a continuous transfer fabric positioned adjacent to the forming fabric to enable the wet web to transfer from the forming fabric to the transfer fabric; (d) means for effecting transfer of the wet web from the forming fabric to the transfer fabric; (e) a rotatable throughdrying cylinder for drying the wet web; (f) a continuous throughdrying fabric which at least partially wraps around the throughdryer and is positioned adjacent to the transfer fabric to enable transfer of the wet web from the transfer fabric to the throughdryer fabric; (g) means for effecting transfer of the wet web from the transfer fabric to the throughdrying fabric; (h) a rotatable reel for winding up the dried web; (i) a reel drum adjacent to the reel for assisting in winding up the dried web; and (j) means for transferring the dried web from the throughdrying fabric to the reel without an open draw.
   In yet one embodiment, the invention resides in the foregoing paper machine wherein the means for transferring the web from the throughdrying fabric to the reel comprises: (a) a continuous first dry end transfer fabric positioned adjacent to the throughdryer fabric to enable transfer of the dried web to the first dry-end transfer fabric;
(b) a continuous loop of a second dry-end transfer fabric positioned adjacent to the first dry-end transfer fabric such that the dried web is sandwiched between the first and second dry-end transfer fabrics, wherein said second dry-end transfer fabric loops around the reel drum and has an air permeability of about 60 m³ per minute per m² (about 200 cubic feet per minute per square foot) or greater; and (c) an air foil positioned within the loop of the second dry end transfer fabric and adjacent to the second dry-end transfer fabric which creates air pressure to maintain the dried web in contact with the second dry-end transfer fabric.

In another embodiment, the invention resides in the foregoing papermaking machine wherein the means for transferring the web from the throughdrying fabric to the reel comprises: (a) a continuous first dry-end transfer fabric positioned adjacent to the throughdryer fabric to enable transfer of the dried web to the first dry-end transfer fabric; (b) a continuous loop of a second dry-end transfer fabric positioned adjacent to the first dry-end transfer fabric such that the dried web is sandwiched between the first and second dry-end transfer fabrics, wherein said second dry-end transfer fabric loops around the reel drum and has an air permeability of about 30 m³ per minute per m² (about 100 cubic feet per minute per square foot) or less.

These and other aspects of the invention will be described in greater detail in reference to accompanying the drawings.

### Brief Description of the Drawing

Figure 1 is a schematic flow diagram illustrating a method for making uncreped throughdried tissue sheets in a manner representative of the prior art using an open draw prior to the reel.
Figure 2 is a schematic flow diagram of a method for making an uncreped throughdried tissue sheet in accordance with this invention utilizing an extended fabric having high permeability.
Figure 3 is a schematic flow diagram of a method for making an uncreped throughdrled tissue sheet in accordance with this invention utilizing an extended fabric having low permeability.
Figure 4 is a plot showing geometric mean tensile strength (GMT) per ply versus the MD tensile strength per ply for a variety of commercial facial tissues, bathroom tissues and towels, as well as several examples produced by the method of this Invention.

### Detailed Description of the Invention

In describing the various figures herein, the same reference numbers are used throughout to describe the same apparatus. To avoid redundancy, detailed descriptions of much of the apparatus described in Figure 1 is not repeated in the descriptions of subsequent figures, although such apparatus is labelled with the same reference numbers.

Referring first to Figure 1, shown is a schematic flow diagram of a representative throughdrying process for making uncreped throughdried tissues. Shown is the headbox 1 which deposits an aqueous suspension of papermaking fibers onto inner forming fabric 3 as it traverses the forming roll 4. Outer forming fabric 5 serves to contain the web while it passes over the forming roll and sheds some of the water. The wet web 6 is then transferred from the inner forming fabric to a wet end transfer fabric 8 with the aid of a vacuum transfer shoe 9. This transfer is preferably carried out with the transfer fabric travelling at a slower speed than the forming fabric (rush transfer) to impart stretch into the final tissue sheet. The wet web is then transferred to the throughdrying fabric 11 with the assistance of a vacuum transfer roll 12. The throughdrying fabric carries the web over the throughdryer 13, blows hot air through the web to dry it while preserving bulk. There can be more than one throughdryer in series (not shown), depending on the speed and the dryer capacity. The dried tissue sheet 15 is then transferred to a first dry end transfer fabric 16 with the aid of vacuum transfer roll 17. The tissue sheet shortly after transfer is sandwiched between the first dry end transfer fabric and a second dry end transfer fabric 18 to positively control the sheet path. The tissue sheet leaves the transfer fabrics and traverses an open draw designated by reference number 20, at which point the sheet is unsupported. The sheet then passes through the winding nip between the reel drum 22 and the reel 23 and is wound into a roll of tissue 25 for subsequent converting, such as slitting, cutting, folding and packaging.

Figure 2 is a schematic flow diagram of process in accordance with this invention, in which the open draw leading to the reel is eliminated. The front end of the process is the same as shown in Figure 1. As the tissue sheet leaves the throughdryer fabric, it is transferred to a first dry end transfer fabric 16 with the aid of a vacuum transfer roll 17. Suitable fabrics for use as the first dry end transfer fabric 16 include, without limitation, a wide variety of fabrics such as Asten 934, Asten 939, Albany 59M, Albany Duotex DD207, Lindsay 543 and the like. The tissue sheet is then compressed between the first dry end transfer fabric and a second dry end transfer fabric 18, which has a greater air permeability than that of the first dry end transfer fabric and which wraps around the reel drum 22. Suitable second dry end transfer fabrics include, without limitation, Asten 960 (air permeability of about 90-120 (about 300-400)), Appleton Mills style Q53F (air permeability of about 120 (about 400)), Appleton Mills style Q53KY (air permeability of about 60 (about 200)), Albany Duotex A81 and Appleton Mills style HC200 (air permeability of about 60 (about 200)). Because of the air flow through the lower fabric caused by roll 31, the sheet transfers to the second dry end transfer fabric 18. It is retained on the top surface of the second dry end transfer fabric by air pressure generated by the presence of an air foil 30 on the underside of the fabric. The tissue sheet is then carried to the winding nip formed between the reel drum and the reel 23 and wound into a roll 25.

Figure 3 respresents another embodiment of the method of this invention, similar to that illustrated in Figure 2 but in which the permeability of the second transfer fabric is much lower than the corresponding fabric used for the method of Figure 2. By lowering the permeability of the second dry end transfer fabric, the need for an air foil is eliminated because with the lower permeability of the second fabric, the sheet tends to naturally adhere to that fabric. At the point of separation the sheet follows the lower permeability fabric due to vacuum action. No air is pumped through the fabric by the various rolls an no foils are required. Suitable low air permeability fabrics for this embodiment include, without limitation, Asten 960 dryer fabric (air permeability of about 15-30 (about 50-100)), COFPA Mononap NP 50 dryer felt (air permeability of about 15 (about 50)) and Appleton Mills dryer felt style H53FH (air permeability of about 22.5 (about 75)).

Figure 4 is a plot showing the geometric mean tensile strength per ply versus MD tensile strength per ply (expressed as grams-force per 3 inches of sample width) for a variety of commercial facial tissues, bathroom tissues and towels, as well as several examples produced by this invention. Numbers "1", "2" and "3" denote commercially available one, two and three-ply facial, bath and towel products. Letters "A-E" refer to tissue products made in Example 1. Data points A and B specifically demonstrate the ability of this invention to consistently produce and reel up tissue webs of low strength. While other low-strength tissues exist, it is commonly known within the industry that their production typically involves reduced machine speed and efficiency. This invention allows the production of such tissues at high speed 914.4 m per minute (3000 feet per minute) or greater) with little, or no, less in efficiency due to dry-end sheet breaks.

### Examples

### Example 1.

In order to further illustrate this invention, several rolls of low strength uncreped throughdried tissue were produced on a commercial tissue machine using the method substantially as illustrated in Figure 1. More specifically, three-layered single-ply bath tissue was made in which the outer layers comprised dispersed, debonded Aracruz eucalyptus fibers and the center layer comprised refined northern softwood kraft fibers, NB-50.

Prior to formation, the eucalyptus fibers were pulped for 15 minutes at 10 percent consistency and dewatered to 30-40 percent consistency. The pulp was then fed to a tiaule shaft disperser operated at 90°C (194°F) with a power input of 3.2 horsepower-days per ton (2.6 kilowatt-days per tonne). Subsequent to dispersing, a softening agent (Berocell 596) was added to the pulp in the amount of 15 pounds of Berocell per tonne of dry fiber (0.75 weight percent).

The softwood fibers were pulped for 30 minutes at 7 percent consistency and diluted to 3.5 percent consistency after pulping, while the dispersed, debonded eucalyptus fibers were diluted to 3.5 percent consistency. The overall layered sheet weight was split 30%/40%/30% among the dispersed eucalyptus/refined softwood/dispersed eucalyptus layers. The center layer was refined to levels required to achieve target strength values, while the outer layers provided the surface softness and bulk. Parez 63INC was added to the center layer at 5.0 kilograms (11 pounds) per tonne of pulp based on the center layer.

A three-layer headbox was used to form the wet web with the refined northern softwood kraft stock in the center layer of the headbox to produce a single center layer for the three-layered product described. Turbulence-generating inserts-recessed about 75 millimeters (3 inches) from the slice and layer dividers extending about 150 millimeters (6 inches) beyond the slice were employed. The net slice opening was about 31 millimeters (1.22 inch), with water flow in the center layer approximately two times that in each outer layer. The consistency of the stock fed to the headbox was about 0.1 weight percent.

The resulting three-layered sheet was formed on a twin-wire, suction form roll, former with forming fabrics (5 and 3 in Figure 1) being Asten 866 and Asten 856 fabrics, respectively. The speed of the forming fabrics was 15.2 meters per second. The newly-formed web was then dewatered to a consistency of about 20-27 percent using vacuum suction from below the forming fabric before being transferred to the transfer fabric, which was travelling at 11.7 meters per second (30% rush transfer). The transfer fabric was an Albany Duotex R-12. A vacuum shoe pulling about 150-380 millimeters (6-15 inches) of mercury vacuum was used to transfer the web to the transfer fabric.

The web was then transferred to a throughdrying fabric (Lindsay Wire T-216-3). The throughdrying fabric was travelling at a speed of about 11.7 meters per second about 2200 feet per minute. The web was carried over a Honeycomb throughdryer operating at a temperature of about 175°C. (350°F) and dried to final dryness of about 98 percent consistency.

The web was then taken to the reel with no opportunity for open draws according to the high permeability fabric scheme illustrated in Figure 2. The first dry end transfer fabric was an Asten 960 while the second dry end transfer fabric was an Albany Duotex A81. The second dry end transfer fabric had an air permeability of 125 m³ per minute per m² (410 cubic feet per minute per square foot) at 1.27 cm (0.5 inch) of water pressure differential. A foil was required under the second dry end transfer fabric at the point of separation of the first and second dry end transfer fabrics. This foil created a low pressure area under the second dry end transfer fabric and caused the sheet to follow this fabric.

Several low strength uncreped throughdried webs were produced at these conditions. All were of approximately 30 grams per square meter in basis weight. Strength parameters were as shown in Table 1.

**TABLE 1**

| | MD Tensile | MD Stretch | CD Tensile | CD Stretch | GMT |
|---|---|---|---|---|---|
| 1-A | 333 | 15 | 185 | 8.9 | 248 |
| 1-B | 388 | 16 | 199 | 9.8 | 277 |
| 1-C | 535 | 18 | 289 | 12.6 | 389 |
| 1-D | 560 | 18.5 | 249 | 9.9 | 373 |
| 1-E | 805 | 20 | 466 | 10.9 | 612 |

This data is represented as points A-E in Figure 4. It illustrates the ability of this invention to conanercially produce and wind tissue webs of low strength.

It will be appreciated that the foregoing examples, given for purposes of illustration, are not to be construed as limiting the scope of this invention, which is defined by the following claims.

## Claims

1. A method for making an uncreped throughdried tissue comprising depositing an aqueous suspension of papermaking fibers onto a forming fabric (3) to form a wet web (6), transferring the wet web (6) to a throughdrying fabric (11), throughdrying the web (6) to form a tissue sheet, and transferring the tissue sheet to a reel (23) such that the sheet does not traverse an open draw while being wound onto the reel (23) in the winding nip formed between the reel (23) and a reel drum (22),
wherein the tissue sheet is:
(a) transferred from the throughdrying fabric (11) to a first dry end transfer fabric (16) using a vacuum roll (17);
(b) carried between the first dry end transfer fabric (16) and the top side of a second dry end transfer fabric (18), the underside of which partially wraps around the reel drum (22);
(c) transferred to the top side of the second dry end transfer fabric (18) and maintained thereon by air pressure created by an air foil (30) positioned on the underside of the second dry end transfer fabric (18); and
(d) wound onto the reel (23), and
wherein the air permeability of the second dry end transfer fabric (18) is about 60 m³ per minute per m² (about 200 cubic feet per minute per square foot) or greater.

2. The method of claim 1 wherein the air permeability of the second dry end transfer fabric (18) is from about 60 m³ per minute per m² to about 150 m³ per minute per m² (about 200 to about 500 cubic feet per minute per square foot).

3. The method of claim 1 wherein the air permeability of the second dry end transfer fabric (18) is from about 90 m³ per minute per m² to about 120 m³ per minute per m² (about 300 to about 400 cubic feet per minute per square foot).

4. A method for making an uncreped throughdried tissue comprising depositing an aqueous suspension of papermaking fibers onto a forming fabric (3) to form a wet web (6), transferring the wet web (6) to a throughdrying fabric (11), throughdrying the web (6) to form a tissue sheet, and transferring the tissue sheet to a reel (23) such that the sheet does not traverse an open draw while being wound onto the reel (23) in the winding nip formed between the reel (23) and a reel drum (22),
wherein the tissue sheet is:
(a) transferred from the throughdrying fabric (11) to a first dry end transfer fabric (16) using a vacuum roll (17);
(b) carried between the first dry end transfer fabric (16) and the top side of a second dry end transfer fabric (18), the underside of which partially wraps around the reel drum (22);
(c) transferred to the top side of the second dry end transfer fabric (18); and
(d) wound onto the reel (23), and
wherein the air permeability of the second dry end transfer fabric (18) is about 30 m³ per minute per m² (about 100 cubic feet per minute per square foot) or less.

5. The method of claim 4 wherein the air permeability of the second dry end transfer fabric (18) is from about 7.5 m³ per minute per m² to about 30 m³ per minute per m²(about 25 to about 100 cubic feet per minute per square foot).

6. The method of claim 4 wherein the air permeability of the second dry end transfer fabric (18) is from about 15 m³ per minute per m² to about 30 m³ per minute per m² (about 50 to about 100 cubic feet per minute per square foot).

7. The method of claim 1 wherein the speed of the tissue sheet is about 600 m per minute (about 2000 feet per minute) or greater.

8. The method of claim 1 wherein the speed of the tissue sheet is about 900 m per minute (about 3000 feet per minute) or greater.

9. A papermaking machine for continuously making an uncreped throughdried paper web comprising:
(a) a headbox (1) for depositing an aqueous suspension of papermaking fibers onto a forming wire;
(b) a continuous forming fabric (3) for receiving the aqueous suspension of papermaking fibers to form a wet web (6);
(c) a continuous transfer fabric (8) positioned adjacent to the forming fabric to enable the wet web (6) to transfer from the forming fabric (3) to the transfer fabric (8);
(d) means (9) for effecting transfer of the wet web (6) from the forming fabric (3) to the transfer fabric (8);
(e) a rotatable throughdrying cylinder (13) for drying the wet web (6);
(f) a continuous throughdrying fabric (11) which at least partially wraps around the throughdryer (13) and is positioned adjacent to the transfer fabric (8) to enable transfer of the wet web (6) from the transfer fabric (8) to the throughdryer fabric (11);
(g) means (12) for effecting transfer of the wet web (6) from the transfer fabric (8) to the throughdrying fabric (11) ;
(h) a rotatable reel (23) for winding up the dried web;
(i) a reel drum (22) adjacent to the reel for assisting in winding up the dried web; and
(j) means for transferring the dried web from the throughdrying fabric (11) to the reel (23) without an open draw,
wherein the means for transferring the web from the throughdrying fabric (11) to the reel (23) comprises:
(a) a continuous first dry end transfer fabric (16) positioned adjacent to the throughdryer fabric (11) to enable transfer of the dried web to the first dry-end transfer fabric (16);
**characterized in that**
(b) a continuous loop of a second dry-end transfer fabric (18) positioned adjacent to the first dry-end transfer fabric (16) is provided such that the dried web is sandwiched between the first and second dry-end transfer fabrics (16, 18), wherein said second dry-end transfer fabric (18) loops around the reel drum (22) and has an air permeability of about 60 m³ per minute per m² (about 200 cubic feet per minute per square foot) or greater; and
(c) an air foil (30) is provided positioned within the loop of the second dry end transfer fabric (18) and adjacent to the second dry-end transfer fabric (18) which creates air pressure to maintain the dried web in contact with the second dry-end transfer fabric (18).

10. A papermaking machine for continuously making an uncreped throughdried paper web comprising:
(a) a headbox (1) for depositing an aqueous suspension of papermaking fibers onto a forming wire;
(b) a continuous forming fabric (3) for receiving the aqueous suspension of papermaking fibers to form a wet web (6);
(c) a continuous transfer fabric (8) positioned adjacent to the forming fabric to enable the wet web (6) to transfer from the forming fabric (3) to the transfer fabric (8);
(d) means (9) for effecting transfer of the wet web (6) from the forming fabric (3) to the transfer fabric (8);
(e) a rotatable throughdrying cylinder (13) for drying the wet web (6);
(f) a continuous throughdrying fabric (11) which at least partially wraps around the throughdryer (13) and is positioned adjacent to the transfer fabric (8) to enable transfer of the wet web (6) from the transfer fabric (8) to the throughdryer fabric (11);
(g) means (12) for effecting transfer of the wet web (6) from the transfer fabric (8) to the throughdrying fabric (11);
(h) a rotatable reel (23) for winding up the dried web;
(i) a reel drum (22) adjacent to the reel for assisting in winding up the dried web; and
(j) means for transferring the dried web from the throughdrying fabric (11) to the reel (23) without an open draw,
wherein the means for transferring the web from the throughdrying fabric (11) to the reel (23) comprises:
(a) a continuous first dry-end transfer fabric (16) positioned adjacent to the throughdryer fabric (11) to enable transfer of the dried web to the first dry-end transfer fabric (16); and
**characterized in that**
(b) a continuous loop of a second dry-end transfer fabric (18) positioned adjacent to the first dry-end transfer fabric (16) is provided such that the dried web is sandwiched between the first and second dry-end transfer fabrics (16, 18), wherein said second dry-end transfer fabric (18) loops around the reel drum (22) and has an air permeability of about 30 m³ per minute per m² (about 100 cubic feet per minute per square foot) or less.

## Patentansprüche

1. Verfahren zum Herstellen eines ungekreppten, durchluftgetrockneten Tissues, umfassend Aufbringen einer wäßrigen Suspension von Fasern zur Papierherstellung auf einen formgebenden Stoff (3) zum Bilden einer nassen Bahn (6), Transferieren der nassen Bahn (6) auf einen Durchlufttrocknungsstoff (11), Durchlufttrocknen der Bahn (6) zum Bilden einer Tissue-Lage, und Transferieren der Tissue-Lage auf eine Rolle (23) derart, daß die Lage keinen ungestützten Bereich unter Zug durchläuft, während sie in dem zwischen der Rolle (23) und einer Rollentrommel (22) ausgebildeten Aufwickelwalzenspalt auf die Rolle (23) aufgewickelt wird,
wobei die Tissue-Lage:
(a) von dem Durchlufttrocknungsstoff (11) unter Verwendung einer Vakuumrolle (17) auf einen ersten Trockenpartie-Transferstoff (16) transferiert wird;
(b) zwischen dem ersten Trockenpartie-Transferstoff (16) und der Oberseite eines zweiten Trockenpartie-Transferstoffs (18), dessen Unterseite teilweise die Rollentrommel (22) umläuft, befördert wird;
(c) auf die Oberseite des zweiten Trockenpartie-Transferstoffs (18) transferiert wird und dort gehalten wird durch Luftdruck, welcher durch ein auf der Unterseite des zweiten Trockenpartie-Transferstoffs (18) angeordneten Luft-Strom (30) erzeugt wird; und
(d) auf die Rolle (23) aufgewickelt wird, und
wobei die Luftdurchlässigkeit des zweiten Trockenpartie-Transferstoffs (18) ungefähr 60 m³ pro Minute pro m² (ungefähr 200 Kubikfuß pro Minute pro Quadratfuß) oder größer ist.

2. Verfahren gemäß Anspruch 1, wobei die Luftdurchlässigkeit des zweiten Trockenpartie-Transferstoffs (18) von ungefähr 60 m³ pro Minute pro m² bis ungefähr 150 m³ pro Minute pro m² (ungefähr 200 bis ungefähr 500 Kubikfuß pro Minute pro Quadratfuß) ist.

3. Verfahren gemäß Anspruch 1, wobei die Luftdurchlässigkeit des zweiten Trockenpartie-Transferstoffs (18) von ungefähr 90 m³ pro Minute pro m² bis ungefähr 120 m³ pro Minute pro m² (ungefähr 300 bis ungefähr 400 Kubikfuß pro Minute pro Quadratfuß) ist.

4. Verfahren zum Herstellen eines ungekreppten, durchluftgetrockneten Tissues, umfassend Aufbringen einer wäßrigen Suspension von Fasern zur Papierherstellung auf einen formgebenden Stoff (3) zum Bilden einer nassen Bahn (6), Transferieren der nassen Bahn (6) auf einen Durchlufttrocknungsstoff (11), Durchlufttrocknen der Bahn (6) zum Bilden einer Tissue-Lage, und Transferieren der Tissue-Lage auf eine Rolle (23) derart, daß die Lage keinen ungestützten Bereich unter Zug durchläuft, während sie in dem zwischen der Rolle (23) und einer Rollentrommel (22) ausgebildeten Aufwickelwalzenspalt auf die Rolle (23) aufgewickelt wird,
wobei die Tissue-Lage:
(a) von dem Durchlufttrocknungsstoff (11) unter Verwendung einer Vakuumrolle (17) auf einen ersten Trockenpartie-Transferstoff (16) transferiert wird;
(b) zwischen dem ersten Trockenpartie-Transferstoff (16) und der Oberseite eines zweiten Trockenpartie-Transferstoffs (18), dessen Unterseite teilweise die Rollentrommel (22) umläuft, befördert wird;
(c) auf die Oberseite des zweiten Trockenpartie-Transferstoffs (18) transferiert wird; und
(d) auf die Rolle (23) aufgewickelt wird, und
wobei die Luftdurchlässigkeit des zweiten Trockenpartie-Transferstoffs (18) ungefähr 30 m³ pro Minute pro m² (ungefähr 100 Kubikfuß pro Minute pro Quadratfuß) oder weniger ist.

5. Verfahren gemäß Anspruch 4, wobei die Luftdurchlässigkeit des zweiten Trockenpartie-Transferstoffs (18) von ungefähr 7,5 m³ pro Minute pro m² bis ungefähr 30 m³ pro Minute pro m² (ungefähr 25 bis ungefähr 100 Kubikfuß pro Minute pro Quadratfuß) ist.

6. Verfahren gemäß Anspruch 4, wobei die Luftdurchlässigkeit des zweiten Trockenpartie-Transferstoffs (18) von ungefähr 15 m³ pro Minute pro m² bis ungefähr 30 m³ pro Minute pro m² (ungefähr 50 bis ungefähr 100 Kubikfuß pro Minute pro Quadratfuß) ist.

7. Verfahren gemäß Anspruch 1, wobei die Geschwindigkeit der Tissue-Lage ungefähr 600 m pro Minute (ungefähr 2000 Fuß pro Minute) oder höher ist.

8. Verfahren gemäß Anspruch 1, wobei die Geschwindigkeit der Tissue-Lage ungefähr 900 m pro Minute (ungefähr 3000 Fuß pro Minute) oder höher ist.

9. Papierherstellungsvorrichtung zum kontinuierlichen Herstellen einer ungekreppten, durchluftgetrockneten Papierbahn, umfassend:
(a) einen Kopfkasten (1) zum Aufbringen einer wäßrigen Suspension von Fasern zur Papierherstellung auf ein formgebendes Sieb;
(b) einen kontinuierlichen formgebenden Stoff (3) zum Aufnehmen der wäßrigen Suspension von Fasern zur Papierherstellung zum Bilden einer nassen Bahn (6) ;
(c) einen kontinuierlichen Transferstoff (8), welcher neben dem formgebenden Stoff angeordnet ist, um Transfer der nassen Bahn (6) von dem formgebenden Stoff (3) auf den Transferstoff (8) zu ermöglichen;
(d) Mittel (9) zum Bewirken des Transfers von dem formgebenden Stoff (3) auf den Transferstoff (8);
(e) einen drehbaren Durchlufttrocknungszylinder (13) zum Trocknen der nassen Bahn (6);
(f) einen kontinuierlichen Durchlufttrocknungsstoff (11), welcher zumindest teilweise den Durchlufttrockner (13) umläuft und neben dem Transferstoff (8) angeordnet ist, um Transfer der nassen Bahn (6) von dem Transferstoff (8) auf den Durchlufttrocknerstoff (11) zu ermöglichen;
(g) Mittel (12) zum Bewirken des Transfers der nassen Bahn (6) vom Transferstoff (8) auf den Durchlufttrocknungsstoff (11);
(h) eine drehbare Rolle (23) zum Aufwickeln der getrockneten Bahn;
(i) eine Rollentrommel (22) neben der Rolle zum Unterstützen des Aufwickelns der getrockneten Bahn; und
(j) Mittel zum Transferieren der getrockneten Bahn von dem Durchlufttrocknungsstoff (11) auf die Rolle (23), ohne Vorhandensein eines ungestützten, unter Zug stehenden Bereichs,
wobei das Mittel zum Transferieren der Bahn von dem Durchlufttrocknungsstoff (11) auf die Rolle (23) umfaßt:
(a) einen kontinuierlichen ersten Trockenpartie-Transferstoff (16), welcher neben dem Durchlufttrockner-Stoff (11) angeordnet ist, um einen Transfer der getrockneten Bahn auf den ersten Trockenpartie-Transferstoff (16) zu ermöglichen;
**dadurch gekennzeichnet, daß**
(b) eine kontinuierliche Schleife eines zweiten Trockenpartie-Transferstoffs (18), welcher neben dem ersten Trockenpartie-Transferstoff (16) angeordnet ist, bereitgestellt ist, so daß die getrocknete Bahn zwischen dem ersten und zweiten Trockenpartie-Transferstoff (16, 18) zwischengelegt ist, wobei der zweite Trockenpartie-Transferstoff (18) die Rollentrommel (22) umläuft und eine Luftdurchlässigkeit von ungefähr 60 m³ pro Minute pro m² (ungefähr 200 Kubikfuß pro Minute pro Quadratfuß) oder größer aufweist; und
(c) ein Luftstrom (30) bereitgestellt ist, welcher innerhalb der Schleife des zweiten Trockenpartie-Transferstoffs (18) und neben dem zweiten Trockenpartie-Transferstoff (18) angeordnet ist und Luftdruck erzeugt, um die getrocknete Bahn in Berührung mit dem zweiten Trockenpartie-Transferstoff (18) zu halten.

10. Papierherstellungsvorrichtung zum kontinuierlichen Herstellen einer ungekreppten, durchluftgetrockneten Papierbahn, umfassend:
(a) einen Kopfkasten (1) zum Aufbringen einer wäßrigen Suspension von Fasern zur Papierherstellung auf ein formgebendes Sieb;
(b) einen kontinuierlichen formgebenden Stoff (3) zum Aufnehmen der wäßrigen Suspension von Fasern zur Papierherstellung zum Bilden einer nassen Bahn (6);
(c) einen kontinuierlichen Transferstoff (8), welcher neben dem formgebenden Stoff angeordnet ist, um Transfer der nassen Bahn (6) von dem formgebenden Stoff (3) auf den Transferstoff (8) zu ermöglichen;
(d) Mittel (9) zum Bewirken des Transfers von dem formgebenden Stoff (3) auf den Transferstoff (8);
(e) einen drehbaren Durchlufttrocknungszylinder (13) zum Trocknen der nassen Bahn (6);
(f) einen kontinuierlichen Durchlufttrocknungsstoff (11), welcher zumindest teilweise den Durchlufttrockner (13) umläuft und neben dem Transferstoff (8) angeordnet ist, um Transfer der nassen Bahn (6) von dem Transferstoff (8) auf den Durchlufttrockner-Stoff (11) zu ermöglichen;
(g) Mittel (12) zum Bewirken des Transfers der nassen Bahn (6) vom Transferstoff (8) auf den Durchlufttrocknungsstoff (11) ;
(h) eine drehbare Rolle (23) zum Aufwickeln der getrockneten Bahn;
(i) eine Rollentrommel (22) neben der Rolle zum Unterstützen des Aufwickelns der getrockneten Bahn; und
(j) Mittel zum Transferieren der getrockneten Bahn von dem Durchlufttrocknungsstoff (11) auf die Rolle (23), ohne Vorhandensein eines ungestützten, unter Zug stehenden Bereichs,
wobei das Mittel zum Transferieren der Bahn von dem Durchlufttrocknungsstoff (11) auf die Rolle (23) umfaßt:
(a) einen kontinuierlichen ersten Trockenpartie-Transferstoff (16), welcher neben dem Durchlufttrockner-Stoff (11) angeordnet ist, um Transfer der getrockneten Bahn auf den ersten Trockenpartie-Transferstoff (16) zu ermöglichen; und
**dadurch gekennzeichnet, daß**
(b) eine kontinuierliche Schleife eines zweiten Trockenpartie-Transferstoffs (18), welcher neben dem ersten Trockenpartie-Transferstoff (16) angeordnet ist, derart bereitgestellt ist, daß die getrocknete Bahn zwischen dem ersten und zweiten Trockenpartie-Transferstoff (16, 18) zwischengelegt ist, wobei der zweite Trockenpartie-Transferstoff (18) die Rollentrommel (22) umläuft und eine Luftdurchlässigkeit von ungefähr 30 m³ pro Minute pro m² (ungefähr 100 Kubikfuß pro Minute pro Quadratfuß) oder weniger aufweist.

## Revendications

1. Procédé de fabrication d'un papier absorbant mince séché par soufflage transversal et non crêpé, comprenant le dépôt d'une suspension aqueuse de fibres papetières sur une toile de formation (3) pour former une nappe humide (6), le transfert de la nappe humide (6) sur une toile de séchage par soufflage transversal (11), le séchage par soufflage transversal de la nappe (6) pour former une feuille de papier absorbant mince, et le transfert de la feuille de papier absorbant mince sur un enrouleur (23) de telle sorte que la feuille ne traverse pas une zone non supportée tandis qu'elle est enroulée sur l'enrouleur (23) dans l'espace d'enroulage formé entre l'enrouleur (23) et un tambour d'enrouleur (22),
la feuille de papier absorbant mince étant :
(a) transférée depuis la toile de séchage par soufflage transversal (11) jusque sur une première toile de transfert côté extrémité sèche (16) en utilisant un rouleau à vide (17) ;
(b) transportée entre la première toile de transfert côté extrémité sèche (16) et la face supérieure d'une seconde toile de transfert côté extrémité sèche (18), dont la face inférieure enveloppe partiellement le tambour d'enrouleur (22) ;
(c) transférée vers la face supérieure de la seconde toile de transfert côté extrémité sèche (18) et maintenue sur celle-ci par la pression de l'air créée par une lame d'air (30) positionnée sur la face inférieure de la seconde toile de transfert côté extrémité sèche (18) ; et
(d) enroulée sur l'enrouleur (23), et
la perméabilité à l'air de la seconde toile de transfert côté extrémité sèche (18) étant d'environ 60 m³/min./m² (environ 200 pieds³/min./pied²) ou davantage.

2. Procédé selon la revendication 1, dans lequel la perméabilité à l'air de la seconde toile de transfert côté extrémité sèche (18) est comprise entre environ 60 m³/min./m² et environ 150 m³/min./m² (entre environ 200 et environ 500 pieds³/min./pied²).

3. Procédé selon la revendication 1, dans lequel la perméabilité à l'air de la seconde toile de transfert côté extrémité sèche (18) est comprise entre environ 90 m³/min./m² et environ 120 m³/min./m² (entre environ 300 et environ 400 pieds³/min./pied²).

4. Procédé de fabrication d'un papier absorbant mince séché par soufflage transversal et non crêpé, comprenant le dépôt d'une suspension aqueuse de fibres papetières sur une toile de formation (3) pour former une nappe humide (6), le transfert de la nappe humide (6) sur une toile de séchage par soufflage transversal (11), le séchage par soufflage transversal de la nappe (6) pour former une feuille de papier absorbant mince, et le transfert de la feuille de papier absorbant mince sur un enrouleur (23) de telle sorte que la feuille ne traverse pas une zone non supportée tandis qu'elle est enroulée sur l'enrouleur (23) dans l'espace d'enroulage formé entre l'enrouleur (23) et un tambour d'enrouleur (22),
la feuille de papier absorbant mince étant :
(a) transférée depuis la toile de séchage par soufflage transversal (11) jusque sur une première toile de transfert côté extrémité sèche (16) en utilisant un rouleau à vide (17) ;
(b) transportée entre la première toile de transfert côté extrémité sèche (16) et la face supérieure d'une seconde toile de transfert côté extrémité sèche (18), dont la face inférieure enveloppe partiellement le tambour d'enrouleur (22) ;
(c) transférée vers la face supérieure de la seconde toile de transfert côté extrémité sèche (18) ; et
(d) enroulée sur l'enrouleur (23), et
la perméabilité à l'air de la seconde toile de transfert côté extrémité sèche (18) étant d'environ 30 m³/min./m² (environ 100 pieds³/min./pied²) ou moins.

5. Procédé selon la revendication 4, dans lequel la perméabilité à l'air de la seconde toile de transfert côté extrémité sèche (18) est comprise entre environ 7,5 m³/min./m² et environ 30 m³/min./m² (entre environ 25 et environ 100 pieds³/min./pied²).

6. Procédé selon la revendication 4, dans lequel la perméabilité à l'air de la seconde toile de transfert côté extrémité sèche (18) est comprise entre environ 15 m³/min./m² et environ 30 m³/min./m² (entre environ 50 et environ 100 pieds³/min./pied²).

7. Procédé selon la revendication 1, dans lequel la vitesse de la feuille de papier absorbant mince est d'environ 600 m/min. (environ 2 000 pieds/min.) ou davantage.

8. Procédé selon la revendication 1, dans lequel la vitesse de la feuille de papier absorbant mince est d'environ 900 m/min. (environ 3 000 pieds/min.) ou davantage.

9. Machine à papier pour la fabrication continue d'une nappe de papier séchée par soufflage transversal et non crêpée, comprenant :
(a) une caisse d'arrivée (1) pour déposer une suspension aqueuse de fibres papetières sur un treillis de formation ;
(b) une toile de formation (3) continue pour recevoir la suspension aqueuse de fibres papetières et former une nappe humide (6) ;
(c) une toile de transfert (8) continue, positionnée adjacente à la toile de formation pour permettre à la nappe humide (6) de passer de la toile de formation (3) à la toile de transfert (8) ;
(d) un moyen (9) pour effectuer le transfert de la nappe humide (6) de la toile de formation (3) à la toile de transfert (8) ;
(e) un cylindre de séchage par soufflage transversal (13) rotatif pour sécher la nappe humide (6) ;
(f) une toile de séchage par soufflage transversal (11) continue qui enveloppe au moins partiellement le séchoir par soufflage transversal (13) et est positionnée adjacente à la toile de transfert (8) pour permettre le transfert de la nappe humide (6) depuis la toile de transfert (8) jusque sur la toile de séchage par soufflage transversal (11) ;
(g) un moyen (12) pour procéder au transfert de la nappe humide (6) depuis la toile de transfert (8) jusque sur la toile de séchage par soufflage transversal (11) ;
(h) un enrouleur (23) rotatif pour enrouler la nappe séchée ;
(i) un tambour d'enrouleur (22) adjacent à l'enrouleur pour aider à l'enroulage de la nappe séchée ; et
(j) un moyen pour transférer la nappe séchée depuis la toile de séchage par soufflage transversal (11) jusque sur l'enrouleur (23) sans zone non supportée,
le moyen de transfert de la nappe depuis la toile de séchage par soufflage transversal (11) jusque sur l'enrouleur (23) comprenant :
(a) une première toile de transfert côté extrémité sèche (16) continue positionnée adjacente à la toile de séchage par soufflage transversal (11) pour permettre le transfert de la nappe séchée vers la première toile de transfert côté extrémité sèche (16) ;
**caractérisé en ce qu'**il est prévu :
(b) une boucle continue d'une seconde toile de transfert côté extrémité sèche (18) positionnée adjacente à la première toile de transfert côté extrémité sèche (16) de telle sorte que la nappe séchée est prise en sandwich entre les première et seconde toiles de transfert côté extrémité sèche (16,18), ladite seconde toile de transfert côté extrémité sèche (18) faisant une boucle autour du tambour d'enrouleur (22) et ayant une perméabilité à l'air d'environ 60 m³/min./m² (environ 200 pieds³/min./pied²) ou plus ; et
(c) une lame d'air (30) positionnée entre la boucle de la seconde toile de transfert côté extrémité sèche (18) et adjacente à la seconde toile de transfert côté extrémité sèche (18), lame qui crée une pression d'air pour maintenir la nappe séchée en contact avec la seconde toile de transfert côté extrémité sèche (18).

10. Machine à papier pour la fabrication continue d'une nappe de papier séchée par soufflage transversal et non crêpée, comprenant :
(a) une caisse d'arrivée (1) pour déposer une suspension aqueuse de fibres papetières sur un treillis de formation ;
(b) une toile de formation (3) continue pour recevoir la suspension aqueuse de fibres papetières et former une nappe humide (6) ;
(c) une toile de transfert (8) continue, positionnée adjacente à la toile de formation pour permettre à la nappe humide (6) de passer de la toile de formation (3) à la toile de transfert (8) ;
(d) un moyen (9) pour effectuer le transfert de la nappe humide (6) de la toile de formation (3) à la toile de transfert (8) ;
(e) un cylindre de séchage par soufflage transversal (13) rotatif pour sécher la nappe humide (6) ;
(f) une toile de séchage par soufflage transversal (11) continue qui enveloppe au moins partiellement le séchoir par soufflage transversal (12) et est positionné adjacent à la toile de transfert (8) pour permettre le transfert de la nappe humide (6) depuis la toile de transfert (8) jusque sur la toile de séchage par soufflage transversal (11) ;
(g) un moyen (12) pour procéder au transfert de la nappe humide (6) depuis la toile de transfert (8) jusque sur la toile de séchage par soufflage transversal (11) ;
(h) un enrouleur (23) rotatif pour enrouler la nappe séchée ;
(i) un tambour d'enrouleur (22) adjacent à l'enrouleur pour aider à l'enroulag de la nappe séchée ; et
(j) un moyen pour transférer la nappe séchée depuis la toile de séchage par soufflage transversal (11) jusque sur l'enrouleur (23) sans zone non supportée,
le moyen de transfert de la nappe depuis la toile de séchage par soufflage transversal (11) jusque sur l'enrouleur (23) comprenant :
(a) une première toile de transfert côté extrémité sèche (16) continue positionnée adjacente à la toile de séchage par soufflage transversal (11) pour permettre le transfert de la nappe séchée vers la première toile de transfert côté extrémité sèche (16) ;
**caractérisé en ce qu'**il est prévu :
(b) une boucle continue d'une seconde toile de transfert côté extrémité sèche (18) positionnée adjacente à la première toile de transfert côté extrémité sèche (16) de telle sorte que la nappe séchée est prise en sandwich entre les première et seconde toiles de transfert côté extrémité sèche (16,18), ladite seconde toile de transfert côté extrémité sèche (18) faisant une boucle autour du tambour d'enrouleur (22) et ayant une perméabilité à l'air d'environ 30 m³/min./m² (environ 100 pieds³/min./pied²) ou moins.
